

1

2,928,718

## METHOD OF BURNING SULPHUR CONTAINING FUELS SUCH AS SHALE

Bjorn Erik Anders Berglund, Hagersten, Hans Olof Horlander, Alvsjo, and John Erik Kjell Svenke, Bromma, Sweden, assignors to Aktiebolaget Atomenergi, Stockholm, Sweden, a Swedish company

No Drawing. Application June 17, 1957  
Serial No. 666,225

Claims priority, application Sweden June 21, 1956

16 Claims. (Cl. 23—1)

The majority of shales contain carbon in a greater or less degree and possibly also organic substances rich in carbon. As a rule such shales are combustible and they are often concentrated to large deposits where the total heat capacity may be very considerable from an industrial point of view. This is for instance the case in Sweden. In all, the Swedish deposits have probably a heat content corresponding to no less than 10,000 million tons of black coal, by way of an estimation.

A plurality of various expedients of utilizing these heat contents have been resorted to. Thus alum shale has been used for a long time as a fuel in kilns for burning limestone into lime. By pyrolysis, the content of organic matters in certain shales is transformed, into hydrocarbons which are gasified and may be condensed and recovered as oil products, the heat content of which then being rendered useful in various ways. This is done, for instance, in the so called shale oil industry which also has succeeded to a certain extent in burning the carbon in the residues, the so-called coke, which are left after the oil has been distilled off so as in this manner to utilize a part of the heat content of the coke.

A simple method of burning completely any combustible contents in shale, shale coke or other shale products would no doubt have very good prospects of being economically applied on an industrial scale for generating hot flue gases for heating purpose, steam or electric power. The use of shale as fuel is hitherto rather moderate due to the fact that procedures employed up to now suffer from technical imperfections and bring in their train severe inconveniences by sulphur dioxide in the combustion gases causing injury and discomfort, the sulphur dioxide being formed in the combustion of the shale material which is rather rich in sulphur.

There is a narrow temperature range within which one has to operate because the spontaneous ignition temperature of the shale is comparatively high, generally well over 600° C., and its sintering temperature is low, about 1000° C. In a molten state the ash is very viscous within a wide temperature interval. For this reason it has not been possible to use combustion methods conventional for fossil fuels or wood. Thus only by controlling the temperature of the combustion zone by means of indirect cooling has one succeeded in carrying through the combustion in some furnace constructions which are in use in the Swedish shale oil industry. In these constructions a relatively coarse material is burnt and the degree of burning out, that is, the utilization of the heat content of the material, is incomplete as is the case in the method stated of burning limestone using shale as a fuel.

A more common utilizing of shale material as a fuel is prohibited, however, by the fact that in methods hitherto current the sulphur content, which generally occurs in shale products and is rather considerable, is transformed

to a great extent into sulphur dioxide which accompanies the flue gases and, upon discharging of the latter into the atmosphere, will cause discomfort and injury. Generally the content of sulphur dioxide in the flue gases, however, is too low to be economically recovered and utilized.

In a procedure according to the present invention a readily controlled, very complete and fast, combustion of the shale material is attained with a moderate excess of air and with no risks of sintering, at the same time as the main portion of the sulphur is bound in the solid combustion residue. The procedure according to the invention is managed in such a manner that the shale material, which is finely divided, preferably to a maximum particle size less than 5 mm., and mixed with a quantity of finely divided alkaline earth metal carbonate, preferably limestone or dolomite, is burnt in a so called fluidized bed with gas mixtures containing air or oxygen, the time of stay at combustion temperature, the quantity and particle size of the limestone or dolomite and the temperature being chosen in such a manner that the content of sulphur dioxide in the flue gases becomes satisfactorily low at the same time as the shale material is comparatively completely burnt out. The necessary conditions for this will become evident from the discussion and experimental results below.

A most important factor is the burning temperature which will be seen from the following trial results obtained in an experimental furnace for burning "fluidized solids," the furnace having a capacity of about 300 kgs. shale per day. Leach residue material from leaching of shale with solutions of sulphuric acid for recovering the uranium content of the shale and having a maximum particle size of 4 mm. was mixed with 23 percent by weight, calculated on the leach residue material, of so called anthraconite, a bituminous limestone (that is, about theoretical quantity, as the lime content of the limestone is about 36% CaO and the sulphur content of the shale material about 6%), the limestone being crushed to a particle size less than 2 mm., whereupon the mixture was burnt in said furnace with an oxygen content in the flue gas of about 6%. The rate of feed was chosen so that the average time of stay became about 50 minutes. At various bed temperatures the SO<sub>2</sub>-content of the flue gas was:

|         | Percent |
|---------|---------|
| 690° C. | 0.30    |
| 800° C. | 0.35    |
| 820° C. | 0.34    |
| 900° C. | 0.42    |

The sulphur contents of the solid residues were then 3-5%. In burning of this shale material under the same conditions but with no admixture of limestone, the sulphur dioxide content in the flue gas was 1.0-1.1%.

The sulphur balance renders the following account of the distribution in the test at 820° C.

|    | Percent of the total amount of sulphur— |                                     |         |
|----|-----------------------------------------|-------------------------------------|---------|
|    | in flue gas                             | in coarse material from the furnace | in dust |
| 65 | 33                                      | 36                                  | 31      |

Generally a temperature exceeding 850° C., with other conditions varied in different ways, has turned out to give too unsatisfactory results as regards the fixing of sulphur. It should be noted that the temperature thus

shall not be raised to values current in burning limestone into lime, that is, exceeding 900° C., which one could be liable to expect with the plausible explanation that the reaction mechanism was first including a dissociation of the calcium carbonate into oxide and thereupon a combining of the sulphur to calcium sulphate. Instead, the reaction shall be conducted at such a low temperature that the vapour pressure of sulphur trioxide in the gas is satisfactorily high. This will not involve the necessity of going down so far in temperature that the combustion can not be carried on spontaneously. Practical trials with Swedish alum shale have shown that the lowest possible temperature for carrying on the combustion in a fluidized bed is about 625° C. A satisfactory fixing of sulphur simultaneously with a good burning out of the shale material takes place at burning temperatures between 625° C. and 850° C., preferably between 700° C. and 800° C. The technique of combustion in a fluidized bed permits operating with a very invariant temperature level—±10° C. without difficulty—and these conditions may hence be very well fulfilled when technically applying the method according to the invention.

The suitable particle size of the shale material is related to several factors, viz. stay time required, gas quantity required for attaining a fluidized state, and the degree of burning out. The method according to the invention can in these respects allow a certain variation but has a demand for the particle size to be within definite limits if a good efficiency is to be obtained. Thus the maximal particle size must be below 6 mm. and preferably below 4 mm. Thus, in performing the method with shale materials having grain sizes below 4-5 mm. and a maximum of the grain size distribution at about 1½ mm., carbon contents in the combustion residue have been attained falling below 0.2%, the starting material having contained 16-18% carbon.

When burning in a fluidized bed, the particle size should preferably be maintained below 4 mm. In order to obtain a larger reaction surface, however, it is advisable to crush the limestone down to below 0.5 mm., but the quantity of the fluidizing air must then be adjusted in such a way that the limestone is not immediately blown out of the furnace without having reacted.

Furthermore, the procedure according to the invention requires, for best results, that the particle size of the limestone material used shall be within definite limits. Too coarse a material has to be added to an unnecessarily great extent compared to what is theoretically necessary in order that the sulphur be fixed during a reasonable stay time of the shale material in the combustion zone. The limestone material should thus be finer than 5-6 mm. and preferably of finer grain than 2-3 mm. An admixture too finely crushed, on the other hand, is not suitable as it will be blown out of the furnace so rapidly that it will not react with the sulphur gas.

The time of stay in the furnace necessary for obtaining the desired effect varies a little with particle size and temperature. Extending the stay time will generally cause the sulphur to be more completely fixed provided that limestone is present in a sufficient quantity. A shorter average stay time than 15 minutes, however, gives an unsatisfactory fixing of the sulphur and preferably the stay time should exceed 20 minutes.

It is worth pointing out that the admixture of limestone does not encumber the process as regards heat economy provided too high an excess is not used. It is true that splitting off carbon dioxide is an endothermic reaction but it is thoroughly compensated by the exothermic combining into sulphate. The reaction

for heating the materials added to the reaction temperature.

In burning shale the oxygen content in the flue gas should be maintained at 3-10%, preferably at 5-8%, so that the reaction  $\text{SO}_2 + \frac{1}{2}\text{O}_2 \rightarrow \text{SO}_3$  is promoted.

As the binding of the sulphur takes place by forming sulphate via sulphur trioxide a rapid arriving at the equilibrium



will act favourably. In burning shale containing sulphur this equilibrium is reached very rapidly as the shale contains iron compounds which are transformed during the burning into iron oxide which acts as a catalyst for said reaction. In fuels which have no such catalytic substance such one may be added if it is found advisable, for instance, in the form of iron oxide.

As has been described above, the presence of dolomite or limestone effects a binding of the sulphur in the burning residues, and, consequently, a decrease of the sulphur contents in the flue gases. According to the invention, it has been found that a further decrease in the sulphur content of the flue gases may be obtained by incorporating small amounts of halogen or halogen compounds in the material during burning. The presence of halogen or halogen compound accelerates the formation of sulphate. As said "catalysts" halogens or halogen compounds are used which under the thermal and chemical conditions in question are transformed into free halogen. For instance, chlorine, sodium chloride, calcium chloride or ferric chloride may be used to advantage.

By investigations it has been proved that the halogen will bring about a more rapid oxidation of sulphur combined as sulphide and also a more rapid dissociation of added carbonate.

#### Example 1

A mixture of a shale leach residue having a particle size below 4 mm. and having different contents of sodium chloride, and 23 percent by weight of bituminous limestone crushed below 2 mm. was burned. The value relates to the  $\text{SO}_2$ -content in the flue gas at an oxygen in the flue gas of 6%.

| Burning temp., ° C. | Addition of NaCl in percent of shale leach residue | Percent $\text{SO}_2$ in the flue gas |      |
|---------------------|----------------------------------------------------|---------------------------------------|------|
|                     |                                                    | 0                                     | 0.33 |
| 800                 | 0                                                  | 0.33                                  | 0.33 |
| 800                 | 1                                                  | 0.23                                  | 0.23 |
| 900                 | 0                                                  | 0.42                                  | 0.42 |
| 900                 | 1                                                  | 0.29                                  | 0.29 |

The sulphur balance will give the following distribution:

|                        | Percent of the total amount of sulphur— |                                     |         |
|------------------------|-----------------------------------------|-------------------------------------|---------|
|                        | in flue gas                             | in coarse material from the furnace | in dust |
| Test, 800° C., 1% NaCl | 23                                      | 46                                  | 31      |
| Test, 900° C., 1% NaCl | 30                                      | 39                                  | 31      |

The addition of common salt then has an effect which substantially exceeds that combining of sulphur which corresponds to combining into sodium sulphate.

#### Example 2

A type of Swedish oil shale was burnt in a fluidized bed at about 750° C., the shale containing 6-7% sulphur. The reaction time was about 35 minutes. When burnt with no additives the shale gave off a flue gas



thus has a heat evolution of 74200 small calories per mols which will yield an excess of heat over that required

with 1.0% SO<sub>2</sub>. Results in accordance with the table below were obtained.

| Admixtures to 100 parts of shale of— |          |       |                   |                                 | Flue gas SO <sub>2</sub> , Percent |
|--------------------------------------|----------|-------|-------------------|---------------------------------|------------------------------------|
| Limestone                            | Dolomite | NaCl  | CaCl <sub>2</sub> | Na <sub>2</sub> SO <sub>4</sub> |                                    |
| 25                                   | -----    | ----- | -----             | -----                           | 1.0                                |
| 25                                   | -----    | ----- | -----             | 2.4                             | 0.65                               |
| 25                                   | -----    | 1     | -----             | -----                           | 0.65                               |
| 25                                   | -----    | 2     | -----             | -----                           | 0.35                               |
| 25                                   | -----    | 4     | -----             | -----                           | 0.2                                |
| 25                                   | 25       | 2     | 2.0               | -----                           | <0.1                               |
| -----                                | -----    | ----- | -----             | -----                           | 0.3                                |
| -----                                | -----    | ----- | -----             | -----                           | 0.45                               |

As shown, addition of compounds containing chlorine in combination with limestone or dolomite has a remarkable effect on the sulphur content in the flue gases.

25 parts of this industrial limestone is equivalent to 7 parts of sulphur. The shale contains 6 or 7% sulphur and therefore a virtually equivalent quantity of lime was used in the example above. There are considerable amounts of limestone interfused in a plurality of shale-deposits, for which reason the costs for the admixture will be small when treating the shale from these deposits. 2% NaCl corresponds to 0.8 part of Na. In combining into Na<sub>2</sub>SO<sub>4</sub>, 0.8 part of sodium correspond to 0.55 part of sulphur. Thus it is evident that the pronounced effect caused by admixing only 2 parts of common salt is not exclusively due to the fact that a chemical combination between sulphur and sodium is formed. Instead the admixture seems to have catalyzed the formation of calcium sulphate.

In the example related above of conducting a procedure according to the present invention the efficiency will depend on the conditions prevailing during the trial, i.e. as regards the time of contact between the gas and the material. Thus at a longer time of contact the same effect will be attained with a less addition of halogen compounds than in the example.

The present invention may to advantage be applied to the burning of limestone in the presence of siliceous material for producing a starting material for hydraulic binders. The sulphur content of the siliceous material will partly be retained in the solid material as calcium sulphate. Generally flue gases are obtained, however, being so rich in sulphur dioxide that they very often can not be directly discharged without considerable inconveniences.

When applying the present invention to this burning of limestone a simple and inexpensive way is offered of transferring a great part of the sulphur to the solid residue by adding a chloride during the burning, for instance CaCl<sub>2</sub>, whereby the content of sulphur dioxide in the flue gas can be brought down to the desired level.

As a matter of course, the cost for the necessary admixture of limestone will depend on the supply of limestone in the neighbourhood of the place where the shale material is utilized by a method according to the present invention. At the Swedish shale deposits, circumstances in this respect are generally extremely favourable as limestone there overlies the shale or is interfused in the same in the form of so called anthraconite. In mining the shale the necessary limestone can thence be obtained simultaneously at a very low cost.

In combustion procedures using a method according to

the present invention the distilled water, for instance, can be used directly for heating by means of hot flue gases, for generating of steam or electric power.

What is claimed is:

- 5 1. A method of burning the combustible constituents of sulphur-containing solid carbonaceous shale materials, comprising intimately mixing the carbonaceous shale material with an alkaline earth metal carbonate in a quantity large enough for binding as sulphate the main part of the sulphur contained in said shale material, heating the resulting mixture in the presence of a catalyst for the oxidation of SO<sub>2</sub> to SO<sub>3</sub>, to initiate combustion of said shale material in a combustion zone in the presence of a gas containing free oxygen, and maintaining the combustion temperature at a temperature, below 900° C., at which no substantial fusion of the resulting ash occurs.
- 10 2. A method as claimed in claim 1, in which the combustion temperature is maintained below 850° C.
- 20 3. A method as claimed in claim 1, in which the combustion temperature is maintained at from 700° to 800° C.
- 25 4. A method as claimed in claim 1, comprising adding to the material to be burned a small amount of a halogen substance selected from the group consisting of elemental halogens and halogen compounds.
- 30 5. A method as claimed in claim 4, in which the amount of halogen substance is not more than 0.2 equivalent halogen per equivalent sulphur.
- 35 6. A method as claimed in claim 4, in which the halogen substance is selected from the group consisting of chlorine, calcium chloride, and sodium chloride.
7. A method as claimed in claim 1, comprising adding combustion air in such an excess that the oxygen content in the flue gas is 3-10%.
- 35 8. A method as claimed in claim 1, comprising adding combustion air in such an excess that the oxygen content of the flue gas is 5-8%.
9. A method as claimed in claim 1, comprising carrying out the combustion in a fluidized bed.
- 40 10. A method as claimed in claim 9, in which the grain size of the solid materials is below 6 millimeters.
11. A method as claimed in claim 10, in which the grain size of the solid materials is below 4 millimeters.
- 45 12. A method as claimed in claim 9, comprising retaining the solid materials in the fluidized bed for an average time of stay of at least 20 minutes.
13. A method as claimed in claim 1 for burning alum shale containing about 5-7% sulphur, comprising burning the shale together with 20-30% of limestone.
- 50 14. A method as claimed in claim 1 comprising using leach residues from the leaching of shale with sulphuric acid solutions as a shale supply.
15. A method as claimed in claim 1, comprising utilizing the heat evolved for generating steam.
- 55 16. A method as claimed in claim 1, in which the sulphur-containing solid materials are associated, in the combustion zone, with iron oxide acting as catalyst on the reaction SO<sub>2</sub> + 1/2 O<sub>2</sub> ⇌ SO<sub>3</sub>.

60 References Cited in the file of this patent

UNITED STATES PATENTS

- |              |         |               |
|--------------|---------|---------------|
| 1,899,808    | Kern    | Feb. 28, 1933 |
| 2,602,019    | O'Dell  | July 1, 1952  |
| 65 2,830,883 | Eastman | Apr. 15, 1958 |

UNITED STATES PATENT OFFICE  
CERTIFICATE OF CORRECTION

March 15, 1960

Patent No. 2,928,718

Bjorn Erik Anders Berglund et al.

It is hereby certified that error appears in the printed specification of the above numbered patent requiring correction and that the said Letters Patent should read as corrected below.

Column 6, line 57, for "materials are" read -- materials  
is --; line 58, for "ison" read -- iron --; same column 6, line  
59, for "SO<sub>2</sub>+½O<sub>2</sub> <> SO<sub>3</sub>." read -- SO<sub>2</sub>+½O<sub>2</sub> ↔ SO<sub>3</sub>. --.

Signed and sealed this 16th day of August 1960.

(SEAL)

Attest:

KARL H. AXLINE  
Attesting Officer

ROBERT C. WATSON  
Commissioner of Patents